

# UNITED STATES PATENT OFFICE.

DESIRÉ DE NAGY, OF LONDON, ENGLAND, ASSIGNOR OF FIFTEEN ONE-HUNDREDTHS TO ALFRED ERNEST KING AND FIFTEEN ONE-HUNDREDTHS TO GEORGE HENRY ODELL, BOTH OF LONDON, ENGLAND.

## MANUFACTURE OF ANILIN DYESTUFFS.

1,250,289.

Specification of Letters Patent. Patented Dec. 18, 1917.

No Drawing.

Application filed June 28, 1917. Serial No. 177,560.

To all whom it may concern:

Be it known that I, DESIRÉ DE NAGY, a subject of the King of Hungary, residing at 10 West Kensington Mansions, London, 5 England, have invented a certain new and useful Manufacture of Anilin Dyestuffs, of which the following is a specification.

This invention relates to the production, either in substance or on the fiber, of valuable dyestuffs, dyeing black, blue and red and their combinations or kindred shades by the oxidation of aromatic amines by using an oxidizing agent not hitherto employed for this purpose.

15 According to this invention the oxidation is carried out by the use of molybdates, instead of the salts of copper, iron, arsenic and vanadium.

20 The dyestuffs obtained by the use of molybdates possess great fastness to light. As an example: A red dye may be obtained by taking the following:

|    |                             |       |
|----|-----------------------------|-------|
| 25 | Hydrochloric acid (18° Bé.) | 5     |
|    | Anilin oil                  | 5     |
|    | Para-nitranilin             | 1     |
|    | Nitrobenzol                 | 2     |
|    | Ammonium molybdate          | 3/100 |

30 These constituents are boiled together and kept at a temperature raised to 200 to 230° C. until the mass is a paste. This paste is then dissolved in hot water and when cool is precipitated with caustic soda.

35 In use, 5 grams of the red dye may be dissolved in 1 liter of hot water at a temperature of 70 to 80° C., and the solution is made slightly acid with acetic acid. The 40 stuff to be dyed is immersed in the bath, the temperature being maintained for about half-an-hour to one hour, and is then rinsed in cold water and allowed to dry.

Apart from the use of molybdates the 45 dye baths are otherwise made up in the usual manner for black, blue and red colors and their combinations or kindred shades.

The following example will illustrate the 50 process in the case of producing black or black-blue color direct on the fiber:

A bath is made up of:

|                                   |        |
|-----------------------------------|--------|
| Chloranilin, <i>o</i> or <i>p</i> | 5      |
| Hydrochloric acid (18° Bé.)       | 25     |
| Ammonium molybdate                | 2/100  |
| Diphenylamin                      | 1/2    |
| Potassium bichromate              | 5      |
| Potassium chlorate                | 1 8/10 |

dissolved in one liter of boiling water. In this bath which is preferably at a temperature of 70° C. silk, wool, or cotton is immersed for an hour without using any mordant. This gives the best result but the operation may be also conducted cold throughout, or the temperature may even be raised to boiling point. The only subsequent treatment of the fibers is to immerse them in dilute caustic soda lye, which gives the best deep black and black-blue shades. The fibers exhibit a much more intense shade which 70 possesses decidedly increased fastness to the action of light.

I claim:

1. An anilin dyestuff mixture comprising aromatic amines and a molybdate. 75
2. An anilin dyestuff mixture comprising aromatic amines and ammonium molybdate.
3. The production of an anilin dyestuff which comprises boiling and heating together constituents comprising aromatic amines and a molybdate, until the mass becomes a paste, dissolving the mass in hot water, and precipitating the product with caustic soda, substantially as set forth. 80
4. The production of dyestuffs on the fiber comprising immersing the material in a bath containing aromatic amines and a molybdate for the oxidation thereof. 85
5. The production of dyestuffs on the fiber comprising immersing the material in a bath containing aromatic amines and ammonium molybdate for the oxidation of such amines. 90
6. The production of black colors direct on the fiber consisting firstly in immersing the material in a bath containing chloranilin, diphenylamin and ammonium molybdate, and secondly in immersing the said materials in a bath of dilute caustic soda lye. 95

DESIRÉ DE NAGY.

Copies of this patent may be obtained for five cents each, by addressing the "Commissioner of Patents, Washington, D. C."